

Aug. 23, 1960

L. G. DEAN ET AL

2,950,236

ELECTROLYTIC PRODUCTION OF MAGNESIUM METAL

Filed June 24, 1957

2 Sheets-Sheet 1



Fig. 1



Fig. 2

INVENTORS.

Lloyd G. Dean  
Charles W. McCutchen  
BY Griswold & Lurdick  
ATTORNEYS

Aug. 23, 1960

L. G. DEAN ET AL

2,950,236

ELECTROLYTIC PRODUCTION OF MAGNESIUM METAL

Filed June 24, 1957

2 Sheets-Sheet 2



Fig. 3



Fig. 4

INVENTORS.

Lloyd G. Dean  
Charles W. McCutchen

BY Griswold & Burdick  
ATTORNEYS

# United States Patent Office

2,950,236

Patented Aug. 23, 1960

1

2,950,236

## ELECTROLYTIC PRODUCTION OF MAGNESIUM METAL

Lloyd G. Dean and Charles W. McCutchen, Lake Jackson, Tex., assignors to The Dow Chemical Company, Midland, Mich., a corporation of Delaware

Filed June 24, 1957, Ser. No. 667,505

2 Claims. (Cl. 204—70)

The invention relates to electrolytes for and methods of electrolytic production of magnesium. It especially relates to molten salt mixtures as electrolytes having a density less than that of molten magnesium and to the method of producing magnesium therefrom.

Magnesium is currently produced on a large scale by the electrolysis of a fused salt bath containing magnesium chloride. The magnesium chloride of such a bath is usually derived from the ocean or brines of deepwells. Some magnesium chloride is derived from the naturally occurring mixed salt, carnallite:  $KCl \cdot MgCl_2 \cdot 6H_2O$ .

These electrolytic baths currently employed have a density greater than that of molten magnesium. Unless the cathode in the bath consist of a molten metal or an alloy which alloys with molten magnesium produced by the electrolysis, the liberated magnesium rises to the surface of the bath and is removed therefrom in recovering the magnesium so produced. The use of an alloying cathode entails a complex subsequent preparatory step to recover the magnesium therefrom and is not economically feasible. In current practice, therefore, the magnesium is permitted to rise to the surface. Since the gaseous products of the electrolysis are also lighter than the bath, and therefore rise to and evolve from the surface, elaborate means for preventing recombination of the magnesium with the evolving gaseous products have been found necessary.

A further difficulty encountered with baths heavier than molten magnesium is that the magnesium, as it collects at the surface of the bath, is exposed relatively unprotected from air which gives rise to a constant threat of burning of the magnesium, particularly at higher operating temperatures. As a result, a significant amount of the liberated magnesium is reoxidized and unrecoverable. Furthermore, the efficiency of known electrolytic methods of producing magnesium has not been satisfactory as shown by the number of kilowatt-hours of energy required to produce a pound of magnesium. This undesirably low efficiency is due largely to the low conductivity of the electrolytic bath used.

In view of the difficulties attendant upon conventional methods of electrolytic production of magnesium, it is a desideratum in the art to provide an improved electrolyte for and method of producing magnesium electrolytically.

We have discovered that by electrolyzing, with a submerged cathode, a fused salt bath, having a density less than that of molten magnesium metal at the temperature

of electrolysis, comprising  $MgCl_2$ ,  $KCl$  and  $LiCl$  wherein the molar ratio of  $MgCl_2$  to  $KCl$  is greater than 1:1 but is less than 3:1 and the molar ratio of  $LiCl$  to the combined molar weights of  $MgCl_2$  and  $KCl$  is greater than 4:2, magnesium metal is produced out of contact with the atmosphere below the surface of the electrolyte in a highly efficient and convenient manner and is recoverable without significant loss.

We prefer to have present in the bath a fluoride of 10 an alkali or alkaline earth metal in an amount up to about 1.5 percent (i.e. about 0.75 to 1.0 percent of the fluoride fraction) by weight of the bath. There may also be present in the bath the chlorides of sodium and calcium up to about 4 percent of each and the chlorides 15 of strontium and barium up to about 2 percent of each by weight.

The magnesium chloride content of the electrolyte is to be at least 5 weight percent because codeposition of lithium with the magnesium at the cathode becomes objectionably excessive at less than 5 percent by weight 20 of magnesium chloride in the electrolyte. On the other hand, the percentage of magnesium chloride is to be no higher than that which will result in the molten magnesium being of greater density than the electrolyte at 25 the temperature of electrolysis. A density differential of at least 0.034 g. per cc. is recommended. If the density of the electrolyte is not at least 0.034 g. per cc. less than the molten magnesium, the magnesium deposition tends to become erratic due to the tendency of 30 some of the magnesium to remain suspended in the electrolyte. The desired density differential is obtained by maintaining the percentage of components of the electrolyte according to the invention.

In the accompanying drawing, 35 Figure 1 is a plan view of an electrolytic cell with which the invention may be practiced.

Figure 2 is a sectional elevation along line 2—2 of Figure 2.

Figure 3 shows graphically the limits of the components 40 of the electrolyte of the invention in molar percentages.

Figure 4 shows graphically the limits of the components of the electrolyte of the invention in weight percentages.

The molar ratio of  $MgCl_2$  to  $KCl$  of 1:1 is 95.2:74.6 45 by weight and the molar ratio of 3:1 is 286.7:74.6 by weight. The molar ratio of  $LiCl$  to  $MgCl_2+KCl$  of 4:2 is 169.6:169.8 by weight or about 50 percent  $LiCl$  when the molar ratio of  $MgCl_2$  to  $KCl$  is 1:1 and is 169.6:180.1 by weight or about 48.6 percent  $LiCl$  when the molar 50 ratio of  $MgCl_2$  to  $KCl$  is 3:1. By referring to Table I below and to Figures 3 and 4 of the drawing, these molar and weight percentages will be made clear.

TABLE I

Percentage composition of electrolyte

[When  $MgCl_2$  is at the Lower Limit, i.e., 5%]

| Molar Ratio of $MgCl_2$ to $KCl$ Is Just Over 1:1 |             |             |                   |               | Molar Ratio of $MgCl_2$ to $KCl$ Is Just Under 3:1 |             |             |                   |               |
|---------------------------------------------------|-------------|-------------|-------------------|---------------|----------------------------------------------------|-------------|-------------|-------------------|---------------|
|                                                   | Molar Ratio | Wt. Percent | Moles Per 100 Gm. | Molar Percent |                                                    | Molar Ratio | Wt. Percent | Moles Per 100 Gm. | Molar Percent |
| $MgCl_2$ Just Over.....                           | 1           | 5.0         | 0.0525            | 2.3           | Just Under.....                                    | 1.5         | 5.0         | 0.0525            | 2.3           |
| $KCl$ .....                                       | 1           | 3.9         | 0.0525            | 2.3           | .....                                              | 0.5         | 1.3         | 0.0175            | 0.7           |
| $LiCl$ .....                                      | 91.1        | 2.1500      | 95.4              | .....         | .....                                              | 93.7        | 2.2100      | 97.0              | .....         |

[When  $LiCl$  is at Lower Limit, i.e., Just Over 4 moles of  $LiCl$  to 2 moles of  $MgCl_2+KCl$ .]

|                         |   |      |       |     |                 |     |      |        |     |
|-------------------------|---|------|-------|-----|-----------------|-----|------|--------|-----|
| $MgCl_2$ Just Over..... | 1 | 28.0 | 0.294 | 16% | Just Under..... | 1.5 | 40.8 | 0.4275 | 25  |
| $KCl$ .....             | 1 | 22.0 | 0.294 | 16% | .....           | 0.5 | 10.6 | 0.1421 | 8%  |
| $LiCl$ Just Over.....   | 4 | 50.0 | 1.179 | 66% | Just Over.....  | 4.0 | 48.6 | 1.146  | 66% |

It is recommended that the percentage of  $MgCl_2$  not be above about 36% nor the  $LiCl$  be below 50% because the adverse effects on cell efficiency of the decreasing conductivity and on cell operation by the increasing density of the electrolyte which accompanies higher than 36%  $MgCl_2$  or lower than 50%  $LiCl$  are appreciable.

By referring to Figures 3 and 4 of the drawing, the molar percentage and weight percentage limits set out in the above table may be readily understood. The shaded area of Figure 3 shows the limits of the components of the electrolyte of the invention in molar percentages. The shaded area of Figure 4 shows the limits of the components of the electrolyte of the invention in weight percentages.

The electrolyte of the invention has a lower viscosity and surface tension than the heavier-than-magnesium electrolytes currently in use. The lower viscosity and surface tension aid in separating the magnesium metal from the electrolyte and sludge.

The electrolyte of the invention having any of the percentage compositions set out hereinabove will show a marked improvement in conductivity over any other electrolytes useful in the production of magnesium known by the inventors to be currently used. However, the electrolyte of the invention which has the highest conductivity and hence greatest efficiency is one having as low a percentage of magnesium chloride as is permitted without objectionable codeposition of lithium and/or potassium with the magnesium.

A portion of the magnesium metal which collects at the cathode may serve as a molten metal cathode which makes a highly efficient contact surface for further recovery of magnesium from the electrolyte. The cell for use in practicing the invention may be of simple design and construction in that no especial provision need be made to keep the chlorine separate from the magnesium produced since the latter is separated from the chlorine by a barrier of electrolyte. The cell is easily operated, requiring a small degree of control since the magnesium metal coalesces well, cell voltage and current remain in a substantially steady state, fire hazard is reduced, and overflow of molten magnesium from the cell is very unlikely. Voltage requirements are lower than for cells employing known electrolytes of greater density than the magnesium being produced because of the higher conductivity of the electrolyte and closer permissible spacing of anode and cathode as a result of reduced likelihood of recombination of magnesium and chloride ions in the submerged region of the anode. The formation of sludge which collects at the bottom of the cell and which is associated with the electrolysis of salts is substantially less than in cells employing known electrolytes. In the production of magnesium by electrolysis, anodes of carbon or graphite are slowly consumed. Electrolysis employing the electrolyte of the invention results in a substantial reduction in anode consumption over methods employing electrolytes of greater density than molten magnesium at the temperature of electrolysis.

The invention then consists of the improved electrolyte and method of producing magnesium therefrom herein fully described and particularly pointed out in the claims, reference being made to the accompanying drawing.

Referring to Figures 1 and 2 of the drawing in detail, there is shown steel shell 1 inclosing refractory furnace setting 2. Iron pot 3, having a flanged rim, is placed in the furnace setting. The pot holds electrolyte 4, formulated in accordance with the invention, and also serves as the cathode of the cell. The top of the cell is provided with ceramic-lined steel cover 5. About the interior of pot 3 is ceramic lining 6 extending from cover 5 downwardly into electrolyte 4 a sufficient distance to fall below the operating level of the electrolyte. This protects the iron pot from interaction with chlorine formed during the electrolysis. Furnace setting 2 contains inlet pipe 7 for introducing heat as from a burner (not shown).

and outlet pipe 8 for egress of combustion gases of the heating burner. In cover 5 is opening 9 for admission of feed and access to the pot. Opening 9 is provided with a removable cover 10. Outlet 11 is provided for egress of chlorine and other gases, if any, formed during electrolysis. Extending through an opening in cover 5 and into pot 3 is anode 12. The degree to which anode 12 extends is controlled by a block and tackle assembly (not shown). Drain assembly 13 including a valve as shown is provided at the lower portion of pot 3. Current leads 14 and 15 are connected to the anode and cathode respectively by suitable terminals 16 and 17 respectively. Packing gland 18 is provided about the anode at the opening in cover 5.

In carrying out the invention, the furnace setting and pot are heated preferably to a temperature above the melting point of magnesium. The heated pot is then charged either with the electrolyte, formulated in accordance with the invention, or its separate ingredients. In charging the pot initially as with the separate ingredients it is advantageous to first introduce the lowest melting point ingredient ( $LiCl$ ) followed by the other ingredients. If desired, the pot may be charged with the electrolyte ingredients in the unmelted state and thereafter melted by heat admitted through inlet pipe 7. After the pot is charged, the electrolyte is brought to a suitable operating temperature above the melting point of magnesium, the electrolyte then being completely molten except for incidental refractory and insoluble impurities normally present in the electrolyte ingredients when not completely removed by previous purification. A generally desirable operating temperature is in the range of about 660° to 900° C.; a preferable temperature range is about 700° to 800° C.

Electrolysis is effected by applying a suitable potential across the anode and cathode of the cell, making the pot the cathode as shown, so as to pass direct current through the electrolyte. The strength of the current is not sharply critical. For example, a current density at the anode in the range of about 3 to 30 amperes per square inch of submerged anode surface may be used. A preferable current density of the anode is 4 to 15 amperes per square inch. Cathode current densities may vary from those of the anode dependent upon operating conditions, e.g., the relative areas of each contacting the electrolyte.

As the electrolysis proceeds, the magnesium liberated at the cathode sinks in the electrolyte and accumulates at the bottom of the cell to form the molten body of magnesium 19. Chlorine is liberated at the anode and rises to the surface of the electrolyte where it is withdrawn from the cell, as through outlet 11. The accumulated molten magnesium may be removed by means of a dipper or a siphon inserted through port 9 or by means of the drain line assembly 13 by opening the valve therein.

When an electrolyte of the invention, for example, one having a composition by weight of about 12%  $MgCl_2$ , 8%  $KCl$ , 1%  $CaF_2$ , and 79%  $LiCl$ , is electrolyzed in a cell similar to that shown in the drawing, at 750° C., having an anode to cathode spacing of 1.5" and a current density of 10 amp./sq. in. at the anode and 8 amp./sq. in. at the cathode and a cell voltage of 4.4 volts, there is obtained a current efficiency at the cathode as high as 80% and a power efficiency of at least 50% when calculated according to the formulae:

65 (1)

$$\frac{\text{Wt. of Mg produced}}{\text{Wt. of Mg possible}} \times 100$$

= percent cathode efficiency according to Faraday's law.

70 (2)

$$\frac{\text{Decomposition voltage, viz., 2.7 for } MgCl_2}{\text{cell voltage}}$$

75  $\times$  percent cathode efficiency = percent power efficiency

It is understood that the cell of Figures 1 and 2 is illustrative of but one form of cell for use in the practice of the invention and that other forms of cells and modifications of that shown may be used with the novel electrolyte according to the method herein described. The design and construction may vary widely. It may be much more complex and elaborate. The cathode and anode may have any of various configurations. Instead of a single anode and cathode, as shown, there may be a plurality of anodes and cathodes. A cell chamber which is lined with an insulating ceramic material and containing a graphite or high-melting non-alloying electrode extending upwardly from the bottom of the chamber may be used. In such a cell, except for the brief start-up period, molten magnesium collecting on the graphite or metal electrode serves as an efficient molten metal cathode. These and other variations will be apparent to those skilled in the art.

Although the invention encompasses any molar ratio of  $MgCl_2$  to  $KCl$  which is greater than 1:1 and less than 3:1 and any molar ratio of  $LiCl$  to  $MgCl_2+KCl$  which is greater than 4:2, with from between 0.5 and 1.5 percent by weight of  $CaF_2$ , the weights usually employed are those set out in Table II below.

TABLE II

| Component      | Preferred Percentage by Weight |
|----------------|--------------------------------|
| $MgCl_2$ ..... | 7 to 25                        |
| $KCl$ .....    | 5 to 20                        |
| $LiCl$ .....   | 70 to 89                       |
| $CaF_2$ .....  | 1.0                            |

The densities illustrative of molten salt baths for the production of magnesium metal according to the invention and the density of molten magnesium are set out in Table III below. The percentage composition of the baths shown in Table III are those percentages designated by dots on Figure 4.

TABLE III

| 5  | Composition of Electrolytes in Percent by Weight |                  |       | Densities of Electrolytes |         |         |
|----|--------------------------------------------------|------------------|-------|---------------------------|---------|---------|
|    | $MgCl_2$                                         | $LiCl+1\% CaF_2$ | $KCl$ | 750° C.                   | 800° C. | 900° C. |
| 10 | 6.8                                              | 90               | 3.2   | 1.47                      | 1.45    | 1.39    |
|    | 10.0                                             | 85               | 5.0   | 1.49                      | 1.47    | 1.42    |
|    | 14.6                                             | 80               | 6.4   | 1.49                      | 1.47    | 1.42    |
|    | 17.0                                             | 75               | 8.0   | 1.50                      | 1.48    | 1.43    |
|    | 20.4                                             | 70               | 9.6   | 1.51                      | 1.49    | 1.44    |
|    | 24.0                                             | 65               | 11.0  | 1.52                      | 1.49    | 1.45    |
|    | 26.2                                             | 60               | 13.8  | 1.52                      | 1.50    | 1.46    |
|    | 30.6                                             | 55               | 14.4  | 1.53                      | 1.51    | 1.46    |
| 15 | 34.0                                             | 50               | 16.0  | 1.53                      | 1.52    | 1.47    |
|    | 100 percent Magnesium Metal                      |                  |       | 1.567                     | 1.557   | 1.518   |

20 Table II shows the densities of various baths from which the differential between the density of the given electrolyte and molten magnesium can be ascertained by subtraction. In the preferred embodiment of the invention the density differential should be 0.034 g. per cc.

25 As the percent of salts other than the essential components of the bath increases, the operating range necessarily narrows since the other salts, e.g.,  $CaCl_2$  or  $NaCl$ , which may be present in the bath are heavier than  $LiCl$ . From the data shown in Table III it is evident that the density differential increases as the temperature is advanced so that slightly higher concentrations of  $MgCl_2$  can be tolerated at higher temperatures.

30 In the electrolysis of the electrolyte of our invention, the magnesium chloride is dissociated, chlorine collecting at the anode and molten magnesium at the cathode. Electrolytes which are illustrative of the electrolyte of the invention are set out in Table IV and examples of the invention employing the electrolytes of Table IV (wherein the electrolyte used agrees in number with the number of the example) to produce metallic magnesium in a cell, similar to that shown in Figures 1 and 2, are set out in Table V.

TABLE IV

Composition of electrolyte

| Electrolyte No. | LiCl         |             | KCl          |             | MgCl <sub>2</sub> |             | $CaF_2$ , Wt. Percent | Molar Ratio, $MgCl_2:KCl$ | Molar Ratio of $LiCl: MgCl_2+KCl$ |
|-----------------|--------------|-------------|--------------|-------------|-------------------|-------------|-----------------------|---------------------------|-----------------------------------|
|                 | Mole Percent | Wt. Percent | Mole Percent | Wt. Percent | Mole Percent      | Wt. Percent |                       |                           |                                   |
| 1.....          | 80.7         | 66.3        | 8.7          | 12.5        | 10.6              | 19.7        | 0.95                  | 1.23                      | 4.17                              |
| 2.....          | 80.9         | 67.0        | 8.7          | 12.7        | 10.3              | 19.1        | 0.90                  | 1.18                      | 4.28                              |
| 3.....          | 81.1         | 66.9        | 8.5          | 12.3        | 10.4              | 19.2        | 0.92                  | 1.22                      | 4.30                              |
| 4.....          | 81.4         | 67.4        | 7.5          | 11.0        | 11.0              | 20.5        | 0.97                  | 1.46                      | 4.38                              |

TABLE V

[Current conditions and results at 800° C. and electrode spacing of 3 inches.]

| Example | Length of Run in Hours | Average Current in Amp. | Average Voltage in Volts | Avg. Current Den., Amp./in. <sup>2</sup> |         | Cathode Current Efficiency | Kwh. per Lb. of Mg. Produced | Conductivity in Mhos |
|---------|------------------------|-------------------------|--------------------------|------------------------------------------|---------|----------------------------|------------------------------|----------------------|
|         |                        |                         |                          | Anode                                    | Cathode |                            |                              |                      |
| 1.....  | 21.96                  | 247                     | 5.55                     | 4.6                                      | 4.9     | 64.1                       | 8.7                          | 4.7                  |
| 2.....  | 14.20                  | 246                     | 5.90                     | 4.5                                      | 4.9     | 78.1                       | 7.6                          | 4.7                  |
| 3.....  | 10.28                  | 246                     | 6.10                     | 4.5                                      | 4.9     | 74.3                       | 8.2                          | 4.7                  |
| 4.....  | 19.94                  | 242                     | 5.65                     | 4.5                                      | 4.8     | 60.7                       | 9.3                          | 4.7                  |

As the magnesium chloride in the electrolyte becomes depleted during the electrolysis, it is replenished either at intervals or continuously to maintain the desired proportion of it in the electrolyte. Also appropriate additions of lithium chloride may be made if needed as shown by routine tests of the electrolyte. A fluoride of an alkali or alkaline earth metal is preferably present in an amount up to 1 percent of the fluoride fraction (F) to facilitate coalescence of the magnesium. Calcium fluoride, lithium fluoride and magnesium fluoride are the fluorides usually employed. Calcium fluoride is preferred and may conveniently be added as fluorite in the preferred range of 1.0 to 1.5 percent of fluoride by weight of the fused bath.

During the electrolysis a small amount of non-metallic insoluble sludge may accumulate at the bottom of the cell. The sludge may be removed either by a dipper as in the case of the magnesium produced or by draining through the drain assembly 13. The fluoride addition already mentioned also aids in setting the sludge which stratifies below the molten magnesium in the cell. De-sludging operations are necessary after protracted operation but less frequently than is now required in current practices.

Melting the magnesium chloride feed and adding the resulting melt to the cell offers certain advantages over its being added as a solid. When added as a solid, especially in large additions, occasionally fairly large portions of unmelted magnesium chloride fall to the floor of the cell and thus temporarily raise the density of the bath near the cathode.

It has been observed that the electrolyte of the invention tolerates a higher percentage of the impurities most frequently found in feed for electrolytic cells for the production of magnesium than do conventional electrolytes. Impurities up to 1 or 2 percent normally present in the feed such as magnesium oxide, and traces of salts and oxides of other metals among which are those of iron, copper, nickel, silicon, manganese, lead, titanium, boron, aluminum, and chromium may be tolerated. Since most of these metals deposit at a lower potential than does magnesium, the specifications of the magnesium to be produced will predetermine the permissible amounts of such metals.

Conductivity of commonly used electrolytes in the production of magnesium is about 2.25 mhos per cc., whereas the conductivity of the electrolyte of this invention is 4.7 mhos per cc. at 800° C. The power efficiency is consequently much better when the electrolyte of higher conductivity is used. Power efficiencies approaching 60 percent are made possible by our invention in contrast to the

power efficiency of about 32 percent which is the efficiency of present electrolytic magnesium production processes. The per pound cost of magnesium is correspondingly reduced by use of our electrolyte. Sludge deposits are less when our electrolyte is employed. If the feed to the bath is anhydrous to the extent of containing only about 0.5 percent water, graphite consumption of the anode is in the low range of 0.015 pound and less of graphite per pound of magnesium produced.

It is apparent that a number of advantages over known electrolytes and methods of using them stem from practicing the invention. Among these advantages are: recovery of the magnesium in a well coalesced mass at the bottom of the cell away from chlorine and oxygen, a molten cathode inherent in the process immediately after electrolysis begins, lower viscosity and surface tension of the electrolyte facilitating separation of the magnesium from electrolyte and sludge and removal from the cell, a smooth and easily controlled operation, simplified cell design, reduced sludge formation, reduced anode consumption, and increased conductivity and power efficiency over electrolytes in current use resulting in a substantial reduction in operating costs.

Having described the invention, what we claim and desire to protect by Letters Patent is:

1. The method of producing magnesium metal electrolytically, employing a cathode submerged in the electrolyte, by electrolyzing magnesium chloride in a molten salt bath at a temperature between 660° and 900° C., said bath consisting essentially by weight of between 7 and 25 percent  $MgCl_2$ , between 5 and 20 percent  $KCl$ , between about 67 and 89 percent  $LiCl$ , and about 1 percent of a fluoride selected from the class consisting of  $CaF_2$ ,  $MgF_2$ , and  $LiF$ , thereby causing magnesium metal to collect at the submerged cathode, and recovering the metal thus produced.

2. The method of claim 1 wherein the temperature of electrolysis is between 700° and 800° C.

#### References Cited in the file of this patent

##### UNITED STATES PATENTS

- |           |                     |               |
|-----------|---------------------|---------------|
| 868,226   | Seward et al. ----- | Oct. 15, 1907 |
| 931,092   | Seward et al. ----- | Aug. 17, 1909 |
| 1,816,972 | Jessup -----        | Aug. 4, 1931  |

##### FOREIGN PATENTS

- |         |                     |                |
|---------|---------------------|----------------|
| 256,241 | Great Britain ----- | Sept. 22, 1927 |
|---------|---------------------|----------------|

##### OTHER REFERENCES

- |    |                                                            |
|----|------------------------------------------------------------|
| 50 | Ser. No. 340,402, Grothe (A.P.C.), published May 18, 1943. |
|----|------------------------------------------------------------|